

## 1

3,843,421

 WROUGHT NICKEL-BASE ALLOY AND  
PRODUCTS THEREOF

Arthur R. Cox, Lake Park, Fla., Paul R. Holiday, Haverstraw, N.Y., and Gary K. Lewis, Riveria Beach, and Sven D. Soderquist, Palm Beach Gardens, Fla., assignors to United Aircraft Corporation, East Hartford, Conn. No Drawing. Filed Oct. 16, 1972, Ser. No. 298,068  
Int. Cl C22c 19/00

U.S. CL. 148—32

3 Claims

## ABSTRACT OF THE DISCLOSURE

A strong nickel-base superalloy is provided which displays good high temperature mechanical properties, including notch ductility, in wrought form when formulated to a very precise composition.

This invention was made in the performance of a contract with the Department of the Air Force.

## BACKGROUND OF THE INVENTION

This invention relates to the high strength nickel-base superalloy field.

In the patent to Bieber 3,061,426 there is disclosed a nickel-base alloy of the  $\gamma$ - $\gamma'$  type which has for some time been extensively used in cast form in gas turbine engine blade applications. In such form, this alloy has been typically formulated to the nominal chemistry consisting of, by weight, 9.5 percent chromium, 15 percent cobalt, 3 percent molybdenum, 4.8 percent titanium, 5.5 percent aluminum, 1 percent vanadium, 0.015 percent boron, 0.06 percent zirconium, 0.17 percent carbon, balance nickel.

As originally developed and utilized, the strength and ductility of the alloy were such that it was practically undeformable and, hence, found application only in precision cast form and found utility only in those applications, such as turbine blades, where cast properties were acceptable. With the generation of the forging process described in the patent to Moore et al. 3,519,503 means were provided whereby the alloy could, if desired, be readily forged, including forging to shapes such as engine discs as well as miscellaneous other forms such as shafts, rings and seals. Because the high temperature strength/low density characteristics are so favorable for aerospace applications, serious consideration was given to the expanded use of the alloy, particularly for engine discs. Unfortunately, the mechanical property criteria applicable to discs differ in some respects from those required in blades and, although satisfactory performance was attained with the conventional alloy in cast form as blading, it was unsatisfactory in wrought form in engine discs.

In a gas turbine engine, the blades are typically retained in fir tree notches machined in the periphery of the disc. The disc must, therefore, not display unacceptable notch sensitivity. For an acceptable disc alloy, the presence of a notch should not result in a decrease in strength at the notch, vis-a-vis the unnotched specimen of the same dimensions as the notch. Preferably, in fact, the distribution of forces and alloy characteristics should be such that notch strengthening is exhibited. Unfortunately, at the usual specification composition the notch strength of the conventional alloy was less than that of the smooth specimen, particularly in the critical 1300°–1400° F. temperature range to which the periphery of the disc may become heated in operation.

Thus, although the alloy could be formed into disc form, the utility in such form was limited.

## SUMMARY OF THE INVENTION

The present invention is directed to a wrought nickel-base superalloy of critical composition and wrought prod-

## 2

ucts produced therefrom, which, upon suitable heat treatment, produces a specific volume of the strengthening  $\gamma'$  phase, typically  $\text{Ni}_3(\text{Al},\text{Ti})$  together with a carbide, including the  $\text{M}_{23}\text{C}_6$ -type carbide, which not only maintains acceptable levels of other mechanical and physical properties but also provides notch strengthening, particularly in the 1300°–1400° F. temperature range.

The wrought alloy is provided at a nominal chemistry of, by weight, 12.4 percent chromium, 18.5 percent cobalt, 3.2 percent molybdenum, 4.3 percent titanium, 5.0 percent aluminum, 0.8 percent vanadium, 0.02 percent boron, 0.06 percent zirconium, 0.07 percent carbon, balance essentially nickel.

Forged products produced to the foregoing chemistry display notch strengthening in the 1300°–1400° F. temperature range with oxidation resistance to at least 1600° F. when heat treated as follows:

- (a) solution heat treatment at about 2050° F. (4 hours) with oil quench;
- (b) stabilization heat treatment at 1600° F. (8 hours) plus 1800° F. (4 hours); and
- (c) precipitation heat treatment at 1200° F. (24 hours) plus 1400° F. (8 hours).

The fully heat treated article is characterized by a  $\gamma'$  volume percentage of about 50–60 percent, preferably about 56 volume percent, as compared to a more typical 70 volume percent in the usual cast alloy chemistry.

 DESCRIPTION OF THE PREFERRED  
EMBODIMENTS

As previously mentioned, the conventional alloy was developed for and used in the production of castings exhibiting high temperature strength and oxidation resistance. The present invention contemplates wrought component applications and has been developed to produce, upon favorable heat treatment, a specific volume of intermetallic precipitates of the  $\gamma'$  and  $\text{M}_{23}\text{C}_6$  types which provide the requisite mechanical properties, including in particular notch strengthening, in the general temperature range of 1300°–1400° F. This is distinct from the criteria and microstructure used for and present in the prior castings and in wrought components formulated to the same composition as such castings.

The composition, which was found to be critical in several essential respects, is as follows, by weight: 11.9–12.9 percent chromium, 18–19 percent cobalt, 2.8–3.6 percent molybdenum, 4.1–4.5 percent titanium, 4.8–5.2 percent aluminum, 0.5–1 percent vanadium, 0.016–0.024 percent boron, 0.04–0.08 percent zirconium, 0.05–0.09 percent carbon, balance essentially nickel.

The full preferred heat treatment specified is as follows.

- (a) solution heat treatment—heat to 2025°–2125° F.  $\pm 15^\circ$ , hold at temperature for 4 hours, oil quench;
- (b) stabilization heat treatment—heat to 1600° F.  $\pm 15^\circ$ , hold for 8 hours, cool to room temperature at a rate equivalent to air cool, heat to 1800° F.  $\pm 15^\circ$ , hold for 4 hours, and cool at a rate equivalent to air cool, and
- (c) precipitation heat treatment—heat to 1200° F.  $\pm 15^\circ$ , hold for 24 hours, air cool, heat to 1400° F.  $\pm 15^\circ$ , hold for 8 hours, and air cool.

Property criteria minimums are typically as follows:

- (a) tensile properties (fully heat treated forgings).

|                                            | Room<br>temperature | 1300° F. |
|--------------------------------------------|---------------------|----------|
| Tensile strength; p.s.i. ....              | 220,000             | 170,000  |
| Yield strength at 0.2% offset, p.s.i. .... | 145,000             | 145,000  |
| Elongation, percent in 4D ....             | 12                  | 12       |
| Reduction of area, percent ....            | 15                  | 15       |

(b) hardness—Brinell 321–414.

(c) stress-rupture (combination smooth/material specimen)—forging held at 1350° F. under continuously applied axial load of 100,000 p.s.i. shall not rupture in less than 23 hours.

(d) creep rupture—with a smooth specimen at 1300° F. and continuously applied axial load of 85,000 p.s.i., time to 0.2% plastic deformation shall average not less than 150 hours with no value below 110 hours.

Table I provides a comparative distributional analysis 10 of the present invention and the conventional composition in terms of their respective physical properties.

The elements such as cobalt and molybdenum which are primarily present in solid solution with the nickel, do not display particular criticality. Similarly, neither boron nor vanadium appear to be particularly critical elements within the context and limits of the invention.

Although the invention has been described in detail in connection with certain examples and preferred embodiments, in its broader aspects it is not limited thereto. Improvements to and departures therefrom may be made within the scope of the appended claims without departing from the principles of the invention and without sacrificing its chief advantages.

TABLE I.—PROPERTY DISTRIBUTION ANALYSIS

|                     | R.T. tensile (k.s.i.)    |       |             |              |                |     |             |              |
|---------------------|--------------------------|-------|-------------|--------------|----------------|-----|-------------|--------------|
|                     | Conventional composition |       |             |              | This invention |     |             |              |
|                     | YS                       | UTS   | Percent el. | Percent R.A. | YS             | UTS | Percent el. | Percent R.A. |
| Mean                | 144.7                    | 227.5 | 18.4        | 16.7         | 157.7          | 225 | 21.4        | 20.9         |
| -1 $\sigma$ (84%)   | 140.5                    | 221.5 | 15.8        | 15.3         |                |     |             |              |
| -2 $\sigma$ (97.5%) | 136.2                    | 215.6 | 13.3        | 13.9         | 147            | 214 | 15.7        | 15.1         |
| Aim                 | 155                      | 220   | 12          | 15           | 145            | 220 | 12          | 15           |

  

|                     | 1,300° F. tensile        |       |             |              |                |       |             |              |
|---------------------|--------------------------|-------|-------------|--------------|----------------|-------|-------------|--------------|
|                     | Conventional composition |       |             |              | This invention |       |             |              |
|                     | YS                       | UTS   | Percent el. | Percent R.A. | YS             | UTS   | Percent el. | Percent R.A. |
| Mean                | 151.4                    | 181.7 | 15.2        | 17.1         | 153.3          | 178.1 | 20.6        | 24           |
| -1 $\sigma$ (84%)   | 148.5                    | 178   | 11.4        | 12.5         |                |       |             |              |
| -2 $\sigma$ (97.5%) | 145.6                    | 174.3 | 7.6         | 8            | 145            | 171.3 | 14.7        | 16           |
| Aim                 | 150                      | 185   | 12          | 15           | 145            | 170   | 12          | 15           |

  

|                     | Stress rupture (smooth)<br>(1350° F./100 k.s.i.) |             |                |                                |                                                   |                      |                                |                 |
|---------------------|--------------------------------------------------|-------------|----------------|--------------------------------|---------------------------------------------------|----------------------|--------------------------------|-----------------|
|                     | Conventional composition                         |             |                |                                | Stress rupture (V-notch)<br>(1350° F./100 k.s.i.) |                      |                                |                 |
|                     | Hrs.                                             | Percent el. | This invention | Conventional composition, hrs. | Invention, hrs.                                   | This invention, hrs. | Conventional composition, hrs. | Invention, hrs. |
| Mean                | 176.5                                            | 7.9         | 26.9           | 11.2                           | 137.5                                             | 40.8                 | 223.7                          | 145.2           |
| -1 $\sigma$ (84%)   | 150                                              | 6.1         |                |                                | 141                                               |                      | 130                            |                 |
| -2 $\sigma$ (97.5%) | 123                                              | 2.5         | 18             | 5                              | 105                                               | 20                   | 36.2                           | 101             |
| Aim                 | 23                                               | 5           | 23             | 5                              | 23                                                | (2)                  | (3)                            | (3)             |

<sup>1</sup> Distribution appears abnormal.<sup>2</sup> Greater than smooth.<sup>3</sup> 150 avg., 110 min.

From the foregoing Table, it will readily be seen that the alloy of the present invention provides the requisite notch strengthening for sensitive forged or extruded components whereas forgings made from the conventional alloy were unacceptably deficient in this regard. This factor alone is determinative of the utility of the alloy in components such as turbine engine discs. And it is only within the criticality limits of the present invention that the necessary properties have been achieved, providing an article having properties never before reproducibly attained.

In the cast alloy previously used, the  $\gamma'$  content has generally been about 70 volume percent or higher. The wrought alloy composition of the present invention provides a microstructure having about 50–60 volume percent of the strengthening  $\gamma'$  phase, with about 56 volume percent appearing optimum. Thus, in the composition of the present invention, the total aluminum plus titanium content of the alloy is especially critical insofar as these elements are the principal determinants of the amount of the  $\gamma'$  phase which is formed.

Further, in the alloy two carbide phases appear present, including a  $\text{Cr}_{23}\text{C}_6$  carbide distributed along grain boundaries and a  $\text{TiC}$  carbide distributed intragranularly. The  $\text{Cr}_{23}\text{C}_6$  carbide precipitated at the grain boundaries is the phase of importance to the present invention for it produces a region of localized plasticity which can undergo microstrain and provide the necessary delay to failures attributable to grain boundary effects. Thus, the carbon content is especially critical in this alloy.

What is claimed is:

1. A wrought nickel-base superalloy article having a nominal chemistry which consists essentially of, about by weight, 12.4 percent chromium, 18.5 percent cobalt, 3.2 percent molybdenum, 4.3 percent titanium, 5 percent aluminum, 0.8 percent vanadium, 0.02 percent boron, 0.06 percent zirconium, 0.07 percent carbon, balance essentially nickel, and characterized by V-notch strengthening in the temperature range of 1300°–1400° F.

2. An article according to claim 1 which is also characterized by a microstructure in the fully heat treated condition exhibiting 50–60 volume percent of a  $\gamma'$  intermetallic phase.

3. An article according to claim 2 wherein the article is a gas turbine engine component.

## References Cited

## UNITED STATES PATENTS

- 3,061,426 10/1962 Bieber \_\_\_\_\_ 75—171  
 3,519,503 7/1970 Moore et al. \_\_\_\_\_ 148—11.5 F  
 3,642,469 2/1972 Ross et al. \_\_\_\_\_ 75—171

70 RICHARD O. DEAN, Primary Examiner

U.S. CL. X.R.

75—171; 148—12.7, 32.5, 162